

Jan. 27, 1931.

E. F. DAVIS

1,789,968

## METHOD OF MAKING SPLINED GEARS

Filed Aug. 7, 1930



INVENTOR.  
*Ernest F. Davis,*

BY

*Hood & Hahn*  
ATTORNEYS

Patented Jan. 27, 1931

1,789,968

# UNITED STATES PATENT OFFICE

ERNEST F. DAVIS, OF MUNCIE, INDIANA

METHOD OF MAKING SPLINED GEARS

## REISSUED

Application filed August 7, 1930. Serial No. 473,647.

The object of my invention is to produce a splined gear having hardened teeth wherein the splined portion is more accurate than has heretofore been considered commercially practical, the production of said gear involving the new and improved method of heat treatment and quenching.

The accompanying drawings illustrate a special carrier and an associated group of 10 gears.

Fig. 1 being an axial section; and

Fig. 2 a cross-section on line 2—2 of Fig. 1.

My invention contemplates the initial production of gears 10 of unhardened material 15 capable of being hardened by a heating and quenching manipulation and these gears have their splined portions produced by a broaching operation which reduces the splined portions to within a few thousandths 20 of the ultimate desired dimensions.

A group of these gears is then assembled upon a carrier 11 formed of a non-oxidizing material having a coefficient of expansion considerably lower than the coefficient of expansion 25 of the gear material and having splines 12 thereon which fit the splined portion of the gears with such a degree of closeness that, when the carrier and its associated group of gears is subjected to the necessary 30 heat treatment, the splined surfaces of the gears will be free to expand and contract under the heat treatment and such that when the heated group is projected into the quenching bath, say a cyanide bath, the flow of the 35 bath into contact with the splined surfaces of the gears will be materially retarded although not entirely prevented.

In order to accomplish this result, I have found that satisfactory results may be produced by using a carrier of chrome-nickel 40 alloy which has a very low coefficient of expansion. This plug is conveniently provided at one end with a retaining flange 14 and at the other end with a perforation 15 through 45 which a sustaining hook may be projected.

In operation a group of the green gears is placed upon the holder. The assembly is then subjected to the necessary heat treatment; and then, suspended from its perforated 50 end, is lowered into the quenching

bath. The quenching results in a hardening of the teeth of the gears to the desired extent and, because of the retarded quenching of the splined portions of the gears, due to the retarded flow of the bath to these portions 55 and the heat of the holder, the splined surfaces of the gears, while hardened sufficiently to meet commercial requirements of these portions of the gear, are not hardened to an extent equal to the teeth. The splined portions of the gears being free to expand and contract under the heat treatment, the teeth are not so distorted as they would be if the splined portions were held against expansion and contraction and undesirable internal stresses are not set up within the bodies 60 of the gears, and the splined portions come out of the bath at a degree of hardness which permits a finishing broaching, which may be accomplished economically, so that the 65 splined portions may be readily finished to the degree of accuracy required.

I claim as my invention:

1. The process of producing splined gears which comprises the formation of a gear of a specified material with the splined surfaces thereof reduced closely to the desired dimensions, the placing of said gear upon a splined holder, the subjection of said holder and gear to a heat treatment, the subjection of the 75 heated holder and the gear to a quenching bath, and the subsequent removal of material at the splined surfaces of the gear to reduce said surfaces to ultimate dimensions, the holder having such dimensions and such 80 coefficient of expansion that the splined surfaces of the gear will be free to expand and contract during heat treatment and such that the flow of quenching bath to said splined surfaces will be retarded but not ultimately 85 prevented whereby the splined surfaces of the gear upon emergence from the quenching bath will be less hard than the teeth thereof, and in condition to permit, as by a broaching operation, the removal of material therefrom for a final finishing operation.

2. The process of producing splined gears which comprises the formation of gears of a specified material with the splined surfaces thereof reduced closely to the desired dimen- 100

sions, the placing of said gear upon a splined holder, the subjection of said holder and gear to a heat treatment, the subjection of the heated holder and gear to a quenching bath, and the subsequent removal of material at the splined surfaces of the gear to reduce said surfaces to ultimate dimensions, the holder being formed of non-oxidizing material and having such dimensions and such coefficient of expansion that the splined surfaces of the gear will be free to expand and contract during heat treatment and such that the flow of quenching bath to said splined surfaces will be retarded but not ultimately prevented whereby the splined surfaces of the gear blank, upon emergence from the quenching bath will be less hard than the teeth thereof and in condition to permit as by a broaching operation, the removal of material therefrom for a final finishing operation.

In witness whereof, I, ERNEST F. DAVIS, have hereunto set my hand at Muncie, Indiana, this 30th day of July, A. D. one thousand nine hundred and thirty.

25 ERNEST F. DAVIS.

30

35

40

45

50

55

60

65